

Nov. 6, 1923.

1,473,284

F. A. FELDKAMP

ELECTRIC FUSE ELEMENT

Filed May 17, 1921



INVENTOR.

Frederick A. Feldkamp,  
BY  
Frautzsch & Richards  
ATTORNEYS.

## UNITED STATES PATENT OFFICE.

FREDERICK A. FELDKAMP, OF NEWARK, NEW JERSEY.

## ELECTRIC-FUSE ELEMENT.

Application filed May 17, 1921. Serial No. 470,434.

*To all whom it may concern:*

Be it known that I, FREDERICK A. FELDKAMP, a citizen of the United States, residing at Newark, in the county of Essex and 5 State of New Jersey, have invented certain new and useful Improvements in Electric-Fuse Elements; and I do hereby declare the following to be a full, clear, and exact description of the invention, such as will enable others skilled in the art to which it 10 pertains to make and use the same, reference being had to the accompanying drawings, and to characters of reference marked thereon, which form a part of this specification.

15 This invention relates to improvements in electrical fuse mediums; and the invention has reference, more particularly, to a novel electrical fuse medium having characteristics adapted to greatly increase the efficiency 20 of the fuse in carrying out the purposes for which it is employed.

In the first place, the characteristics to be desired in an electrical fuse are, that the same provides a medium of the highest possible conductivity, and that the medium also possesses a comparatively low melting point. 25 Unfortunately said desirable characteristics can not both be provided by any known single elementary metal, nor can the same be provided to the highest degree by any form 30 of metallic alloy. For example, copper, being highly conductive, would answer the first requirement, but copper possesses a comparatively high melting point, not fusing until after it is brought to a bright red 35 heat, its melting point being above 1000° C. Metals or alloys which would answer the second requirement, to wit, possession of a comparatively low melting point, are all 40 comparatively poor conductors. I have found that a fuse medium of a composite nature having its elements relatively disposed in a peculiar intimate combination and manner, serves to best provide, in a high 45 degree, both the desired characteristics of high specific conductivity and comparatively low melting point.

It is, therefore, the purpose and object of 50 this invention to provide a fuse medium of a composite nature, which will best afford, in operation, both high specific conductivity and a comparatively low melting point. To this end the invention comprises a fuse medium consisting of a main metallic body of

high specific conductivity, such, for example, 55 as copper, to the surface of which is applied an overlying intimately united portion of another metal or metallic alloy possessing a comparatively low melting point, such, for example, as cadmium or an alloy containing 60 cadmium. I find it preferable to apply the overlying portion to the main body at a point or points intermediate the ends of the latter, although I do not limit myself entirely to such spot or point location thereof. 65 The appearance and mechanical relations of the above mentioned elements making up my novel fuse medium is clearly illustrated in the accompanying drawings, in which:—

Figure 1 is a side elevation of a fuse wire 70 made according to and embodying the principles of this invention; Figure 2 is a longitudinal section of the same, taken on line 2—2 in Figure 1, the main body being shown in elevation with the portions applied 75 thereto shown in section; Figure 3 is a transverse longitudinal section of the same, taken on line 3—3 in Figure 2, the main body being therein also shown in elevation with the portions applied thereto shown in section. 80

Figure 4 is a side elevation of a slightly modified form of the novel fuse wire embodying the principles of my invention.

Figure 5 is an enlarged detail longitudinal section, showing a portion of the main body 85 in elevation, and the portion applied thereto in section.

Figure 6 is a face view of a fuse strip made according to and embodying the principles of my invention; Figure 7 is an edge 90 view of the same; and Figure 8 is a longitudinal section through the same, taken on line 8—8 in said Figure 6.

Similar characters of reference are employed in all of the above described views, 95 to indicate corresponding parts.

Referring now to the drawings, the reference character 1 indicates the main body of a fuse medium in a wire or cylindrical form. This main body is preferably made of copper, which possesses high specific conductivity. Combined or united with the surface of said main body 1 throughout its length or at one or more points intermediate its ends, is an overlying portion 2 comprised of a 100 metal having the property of readily alloying with copper at comparatively low temperatures, when intimately united with the

surface of the latter; while at the same time being itself possessed of a comparatively low melting point. A metal desirable for use as such overlying portion 2 is cadmium, which 5 may be employed alone in its pure state, but which is preferably formed into an alloy with tin, since the presence of the tin serves to more readily unite the portion 2 to the surface of the body 1 when applied thereto. 10 The operation of application being in the nature of a soldering process, whereby the contiguous surfaces of the copper and overlying cadmium or cadmium alloy are intimately united together. The intimate adherence of one metal with the other thus produced is essential to the carrying out of the principles involved in my invention, since such relation prevents any oxidation or tarnishing of the meeting surfaces, so that 15 when the fuse medium is subjected to excess temperature oxidation is eliminated with the result that the component elements of the fuse medium may alloy together, thereby decreasing the melting point and increasing 20 the resistance of the fuse as a whole, both of which factors tend to accelerate the reduction of the same to the "blowing" point.

Since most fuse wires are usually supported within cartridge containers, which 30 in use occupy a vertical position, so that the fuse wire itself is perpendicularly disposed, it is desirable to provide means for preventing the applied portions 2 from becoming detached or displaced from their position 35 relative to the main body 1, when the same begin to flux or melt in operation. To this end the said main body or wire 1 is provided with a flattened out portion 3 at the point of application of the portion 2, which 40 forms a seat or socket for retaining the latter against dislocation when the same becomes fluid; the retention effect being in the nature of capilarity.

The operation of the composite fuse medium, constructed as above described, is as follows:—

At ordinary current load or permitted overloads, according to the selective capacity and rating of the fuse medium, the overlying portion 2 of cadmium or cadmium alloy, remains inactive and rigid or unfluxed, while the current flows through both elements of the composite fuse. When, however, the fuse is subjected to an excessive current overload, the temperature of the fuse rises accordingly, and the overlying portion 2 of cadmium or cadmium alloy becomes highly active, that is, it fluxes or melts, and while so doing it forms a combination 55 or new alloy by alloying or combining with the copper comprising the main body or wire 1. This alloying reaction between the two elements of the composite fuse medium begins while the copper element is still at a comparatively low temperature. The alloy-

ing reaction when set up results in producing, at the point or points occupied by the overlying portions 2, a metallic combination or alloy of copper and cadmium or cadmium alloy which possesses both a lower 70 melting point and a higher resistance than is possessed by the copper alone, consequently after initiation of such alloying reaction there is a tendency to accelerate the "blowing" of the fuse medium at the point 75 or points where such alloying reaction occurs. The reason for this is that the heat generation will be increased at such point or points due to the progressively increasing resistance caused by the progress of the alloying process, until such a state is reached that all of the underlying copper is converted into a lower melting point alloy, whereupon the fuse medium will "blow" at 80 such point or points.

It will thus be apparent that the novel fuse medium provides for a normal condition of high specific conductivity whereby normal current loads and permitted overloads may be conducted therethrough without reaction between the component parts, and yet the same is adapted, under abnormal increases of temperature due to excessive current overload, to melt, fuse or "blow" at a comparatively low temperature, 90 thereby eliminating the danger of carbonizing the cartridge container in which such fuse mediums are usually disposed, due to accumulative excesses of temperature immediately preceding the "blowing" of the same. 95 Another advantage afforded by my novel construction of fuse medium is that it permits, by reason of the high specific conductivity of the main body 1 or copper element, 100 a reduction of the amount or mass of metal required for the fuse and necessary to carry the specified current load, thereby reducing the pressure, within a cartridge containing the fuse medium, at the moment of "blowing", by reason of the correspondingly reduced volume of gases generated by the vaporization of the lesser amount of metal required for my novel fuse medium.

Referring now to Figures 6 to 8 inclusive of the accompanying drawings, I have shown the principles of my invention as applied to a fuse medium of the flat strip type. In said views, the reference character 4 indicates a strip or flat main body of metal possessing high specific conductivity, such as copper. This strip or flat main body 4 is provided at a point or points intermediate its ends with a plurality of perforations 5. The reference character 6 indicates an applied over-lying portion of metal or metallic alloy adapted to combine itself with the main body 4 at the point of application thereto under an excess of normal permitted temperature, at the same time said over-lying portion possesses a comparatively low 110 115 120 125 130

melting point, preferably said overlying portion 6 being made of cadmium or cadmium alloy. When applying said over-lying portion 6 to the strip or flat body portion 4, 5 the same is caused to flow over the perforate portion of the latter so that parts thereof, such as the projections 7, enter and imbed themselves in the perforations 5, whereby the said over-lying portion 6 is retained in 10 mechanically secured relation to the strip or main body 4 against dislocation therefrom when fluxing.

In use and operation the above described strip type of fuse medium functions in the 15 same manner and to the same advantage, as does the wire type of fuse medium as heretofore described.

I am aware that besides cadmium or cadmium tin alloys, there are other metals or 20 combinations of metals for use as the over-lying portions of low melting point character-istics for the fuse medium which would have the tendency of alloying with copper at a comparatively low temperature, hence, 25 broadly my invention contemplates the em-ployment of any metal or metallic alloy which will thus function.

I am also aware that composite fuse me-diums of various kinds have also been here- 30 tofore known, but I wish to distinguish my present invention from all such by the prin-ciple of its structure which requires the ap-plication of the overlying portion of the fuse medium to the main body to be of such 35 character that the meeting surfaces of the two elements unite in that close mutual ad-herence necessary to prevent oxidation and to permit the alloying reaction above ex-plained to be initiated when the medium is 40 subjected to excessive temperature.

I claim:—

1. An electric fuse of high specific con-ductivity and comparatively high melting point in intimate closely adhering contact with 45 a superimposed metallic material which un-der normal temperature is inactive and un-der excessive higher temperature combines with the fuse material to form an alloy of lower melting point.

50 2. An electric fuse medium comprising a metallic main body of high specific con-ductivity and comparatively high melting point having united to its surface a metallic over-lying portion possessing a comparatively low melting point and of a character adapted to 55 form an alloy with said main body by the action of heat generated under excessive cur-rent overload passing through said fuse me-dium.

60 3. An electric fuse medium normally of high specific electrical conductivity, means providing a "blowing" zone intermediate the ends thereof, said means comprising an over-lying portion of metallic material united 65 with said fuse medium adapted by the ac-

tion of heat generated under a current over-load to combine with the underlying por-tion of said fuse medium to form an alloy therewith tending to increasingly reduce the conductivity and lower the melting point 70 thereof.

4. In an electric fuse medium, the com-bination with a main body of metal of high specific conductivity of an overlying metallic portion united therewith at a point thereof 75 intermediate its ends, said overlying metal-lic portion being adapted by the action of an excess of heat above a normal permitted temperature to combine with the under-lying portion of said main body to form an 80 alloy therewith tending to both increase the resistance and lower the melting point of the fuse at such points.

5. In an electric fuse medium, the com-bination with a main body of metal of high specific conductivity of an overlying metallic portion united therewith at a point thereof intermediate its ends, said overlying metal-lic portion being adapted by the action 85 of an excess of heat above a normal per-mitted temperature to combine with the under-lying portion of said main body to form an 90 alloy therewith tending to reduce the conductivity and lower the melting point of the latter, and means for retaining said overlying metallic portion against displace-ment when fluxed.

6. An electric fuse medium comprising a main body of copper having united therewith at one or more points intermediate its 100 ends an overlying portion of metallic mate-rial adapted by the action of abnormal heat to form an alloy with the underlying copper body tending to both increase the resistance and lower the melting point of the latter 105 whereby the "blowing" of the fuse medium rapidly follows and is localized at said point or points thereof.

7. An electric fuse medium comprising a main body of copper having united therewith at one or more points intermediate its 110 ends an overlying portion of metallic mate-rial adapted by the action of abnormal heat to form an alloy with the underlying copper body tending to both increase the resistance and lower the melting point of the latter 115 whereby the "blowing" of the fuse medium rapidly follows and is localized at said point or points thereof, and means for retaining said overlying metallic portion against dis-placement when fluxed.

8. An electric fuse medium comprising a main body of copper having applied thereto an overlying portion of cadmium intim-ately united with its surface, as and for the pur- 125 poses set forth.

9. An electric fuse medium comprising a main body of copper having applied thereto an overlying portion of cadmium intim-ately united with its surface, as and for the pur- 130

poses set forth, and means for preventing dislocation of said cadmium when fluxed.

10. An electric fuse medium comprising a main body of copper having applied thereto an overlying portion of cadmium alloy intimately united with its surface, as and for the purposes set forth.

In testimony that I claim the invention set forth above I have hereunto set my hand this 16th day of May, 1921.

FREDERICK A. FELDKAMP.

Witnesses:

FRED'K C. FRAENTZEL,  
EVA E. DESCH.